

Sept. 8, 1953

F. F. GANS  
MANUFACTURING PROCESS OF CADMIUM  
SULFIDE, SELENIDE, TELLURIDE  
PHOTOCONDUCTING CELLS  
Filed Nov. 10, 1952

2,651,700



INVENTOR  
FRANCOIS F. GANS  
By  
Wendoverth Lind & Ponack  
ATTORNEYS

## UNITED STATES PATENT OFFICE

2,651,700

MANUFACTURING PROCESS OF CADMIUM  
SULFIDE, SELENIDE, TELLURIDE PHOTO-  
CONDUCTING CELLS

François F. Gans, Paris, France

Application November 10, 1952, Serial No. 319,650  
In France November 24, 1951

5 Claims. (Cl. 201—63)

**1** The present invention relates to a process for the production of photoelectric cells, and more specifically cadmium sulfide photoconducting cells, i. e. cells the electrical resistance of which varies according as they are exposed to radiation.

It has been noticed that the cadmium sulfide becomes the more efficient as suitably selected impurities called "activators" are added in small quantities to its crystal lattice. These activators are very numerous and it may be mentioned copper, silver, gold, lead and nickel, etc.

It has also been noticed that cadmium selenide and cadmium telluride present similar properties.

The described procedure relates to cadmium sulfide but it is to be understood that it applies equally to both cadmium selenide and cadmium telluride cells, without departing from the spirit of the invention.

In order to produce cadmium sulfide photoconducting cells, a standard process is to dip a cadmium sulfide crystal, or a slip of such material as glass on which a layer of cadmium sulfide has been evaporated, into a homogeneous mixture of cadmium sulfide and of the chosen activator or activators, reduced into a fine powder. Then the vessel containing the powder is heated at a suitable temperature of 500° C. Thermodiffusion produces an equilibrium between the activator content of the crystal, or of the evaporated layer on the one hand, and of the mixture on the other.

Such processes are not without drawbacks. The crystals are fairly difficult to prepare, their size is seldom large enough, seldom more than one centimeter, their thickness is always very small, less than one millimeter, and their brittleness makes them difficult to handle.

The dimensions of the evaporated layers may be large, but they are very thin; they take a long time to prepare, and, therefore, their price is high. Besides, the evaporated layers have a lacunary structure and, owing to this structure, there appears, in series with the resistance that varies according to the illumination, a parasitic resistance independent from the illumination which results in a diminution of the sensibility of the cell. On the other hand, the resistance opposed by the lacunae of the layer to the current is not regular, and it results into a parasitic noise which adds itself to the photoelectric signal given by the cell.

According to the process the present invention relates to, process which is disclosed in relation with the figure which represents a press,

**2** these drawbacks are avoided by producing, through compression and sintering of a very finely ground powder, a cell the compactness of which may be compared to that of crystal, but which may possess any size.

In order to produce the above mentioned cell, the following procedure is used.

The mixture of cadmium sulfide and of the activator or activators is ground and homogenized for several days into a very fine powder (by such an apparatus as a ball-mill) so that the grains of the powder should have a diameter of under 5 $\mu$  or thereabout.

In order to give a clearer idea of the nature and contents of the activating powders, three examples are given hereinafter.

Example No. 1: Cells of great inertia in the neighbourhood of one second and of sensibility in the neighbourhood of 5 to 10 a./lm. (amperes per lumen)

|    |      |       |      |
|----|------|-------|------|
| 15 | CdS  | ----- | 1000 |
|    | CuS  | ----- | 4    |
|    | CdSe | ----- | 20   |
| 20 | Te   | ----- | 20   |

Example No. 2: Ordinary cells of average inertia and sensibility (inertia of about 1/100 second and sensibility of about one ampere per lumen):

|    |                   |       |      |
|----|-------------------|-------|------|
| 30 | CdS               | ----- | 1000 |
|    | CuS               | ----- | 2.5  |
|    | NiCl <sub>2</sub> | ----- | 5    |
| 25 | CdSe              | ----- | 30   |

Example No. 3: Cells of low inertia of about 1/1000 second and sensibility of about 0.1 to 0.5 a./lm.

|    |                   |       |      |
|----|-------------------|-------|------|
| 35 | CdS               | ----- | 1000 |
|    | CuS               | ----- | 3    |
|    | NiCl <sub>2</sub> | ----- | 25   |

Once the powder has been obtained, a certain quantity of said powder, 0.1 to 1 gramme, is taken to a housing 3, having a surface of a few cm.<sup>2</sup>, of a press that can produce a very high pressure of over 2 tons per cm.<sup>2</sup>.

This press includes a piston that moves in a cylinder 2 at the bottom of which is the housing of the powder 3. To avoid the effects of the gas contained between the grains of powder, the cylinder of the press communicates through a pipe 4 with a vacuum pump sketched in 5.

6 is an electric heater which makes it possible to heat at a temperature between 550° and 600° C. the tablet of powder while the pressure is being applied to it.

## 3

The electrodes are brush painted with a conducting silver lacquer such as the one sold by the firm Degussa under No. 200.

The sensibility of the cells depends on the pressure as shown by the following table which gives in megohms, the resistance of two cells manufactured with the powder of Example No. 2.

Cell I compressed up to 8 tons per cm.<sup>2</sup>  
Cell II compressed up to 15 tons per cm.<sup>2</sup>

| Illumination in lux               | 25  | 50 | 100  | 200  | 500  | 1,000 |
|-----------------------------------|-----|----|------|------|------|-------|
| resistance of cell I in meg-ohms  | 100 | 50 | 15   | 2.4  | 1.6  | 1-    |
| resistance of cell II in meg-ohms | 4.5 | 1  | 0.45 | 0.16 | 0.12 | 0.1   |

What I claim is:

1. A process for the production of photoelectric cells containing a photoconducting material selected from the class consisting of cadmium sulfide, cadmium selenide and cadmium telluride comprising mixing said photoconducting material with activators therefor, grinding the mixture to obtain a powder having a particle diameter

of not greater than about 5  $\mu$ , and compressing and heating said powder under a pressure of about 2 tons per square centimeter and a temperature of about 550° C. to obtain said powder in tablet form, said tablet adapted to be provided with conducting electrodes.

2. A process as in claim 1 wherein said pressure is about 15 tons per square centimeter and said temperature is between about 550° C. and 600° C.

10 3. A photoconducting cell comprising particles of a photoconducting material selected from the class consisting of cadmium sulfide, cadmium selenide and cadmium telluride and an activator therefor, ground to a particle size of less than about 5  $\mu$  compressed under a pressure of more than about 2 tons per square centimeter and heated to a temperature of above 550° C.

4. The structure of claim 3 provided with conducting electrodes.

20 5. The structure of claim 4 in which the electrodes are coatings of metal conducting lacquer

FRANCOIS F. GANS.

No references cited.